

## UNITED STATES PATENT OFFICE

2,035,490

## REMOVAL OF WAX FROM HYDROCARBON OIL

Bernard Y. McCarty, Beacon, N. Y., and William E. Skelton, Fort Worth, Tex., assignors to The Texas Company, New York, N. Y., a corporation of Delaware

No Drawing. Application June 8, 1934,  
Serial No. 729,600

4 Claims. (Cl. 196—19)

This invention relates to the removal of wax from hydrocarbons and more particularly to an improved process for the removal of paraffin from lubricating oil fractions derived from petroleum.

5 This application is a continuation-in-part of our copending application, Serial No. 578,206, filed November 30, 1931, now Patent No. 1,995,153, issued March 19, 1935, for Removal of wax from hydrocarbon oil.

10 The invention contemplates a process of dewaxing wax-containing lubricating oil fractions by filtration at low temperatures, wherein the wax-containing oil is mixed with a wax-precipitating liquid medium composed of a solvent liquid 15 or mixture of solvent liquids which is completely miscible with, and exerts a substantially complete solvent action upon, the oil at the temperatures at which the wax constituents are precipitated from the oil in solid form and which has substantially no solvent action on the solid hydrocarbons at such temperatures. The resulting mixture is then chilled to precipitate the solid hydrocarbons which are removed by filtration.

More specifically the invention contemplates 25 mixing with lubricating oil fractions a wax-precipitating liquid medium composed of a mixture of ortho-dichloro-benzene with either amyl alcohol, ethylene-glycol-mono-ethyl-ether, diethylene-glycol-mono-butyl ether, methyl ethyl ketone, propylene dichloride or ethylene dichloride. In some instances, ordinary commercial benzene 30 may be used as in the case of mixtures with the ether compounds.

An object of this invention is to effect dewaxing of paraffin-containing hydrocarbon oils 35 with an improved type of solvent liquid composed of a mixture of solvents having selective solvent properties between the oil and the wax constituents and which, in addition, retains its selective solvent properties at relatively low temperatures whereby the precipitation of the wax from the mixture, particularly in the case of mixtures with relatively viscous oils, is effected in a more readily filterable form. At the same time, a high 40 yield of dewaxed oil is obtained.

45 A further object has been to develop a solvent liquid which possessed the foregoing properties at relatively low temperatures and which is, therefore, adaptable for the manufacture of lubricating oils having pour tests of  $-20^{\circ}$  F. and lower.

50 A selective solvent suitable for the foregoing dewaxing operation, and particularly when composed of two or more organic solvents, must retain its homogeneity and its property of remain-

ing completely miscible with the liquid hydrocarbon constituents of the mineral oil at temperatures substantially well below  $0^{\circ}$  F. Complete miscibility is necessary in order to prevent separation of such liquid hydrocarbons from the 5 solution. Such separated liquid hydrocarbons materially increase the viscosity of the solution thereby tending to reduce the filtering rate to a point where the operation is not economical. In addition, the presence of this separated liquid 10 gives rise to a condition which is productive upon filtration of a wax cake containing substantial amounts of oil so that the maximum yield of dewaxed oil is not realized.

It is essential that such a solvent mixture remain 15 completely homogeneous at these low temperatures and not exhibit any tendency for any of its components to separate from the mixture. Upon separation of one of the components from the solvent mixture, the ratio of the components 20 remaining in the mixture is altered, thereby changing its selective solvent properties so that the wax constituents will not be completely precipitated and/or appreciable amounts of the liquid hydrocarbon may separate from the solution 25 due to the resulting lack of complete miscibility on the part of the solvent with the oil owing to its altered condition.

Extensive investigation has demonstrated that 30 a solvent liquid or solvent mixture satisfactory for use as a wax-precipitating medium in the dewaxing of wax-containing hydrocarbon oils must possess, among other things, low absolute viscosity and low viscosity temperature coefficient, high oil solubility at low temperatures, low 35 wax solubility at low temperatures, low freezing point, and also possess the property of precipitating wax in a readily filterable condition.

Accordingly after investigating various solvent 40 liquid mixtures it has been found that a mixture of ortho-dichloro-benzene and amyl alcohol, ethylene-glycol-mono-ethyl ether, diethylene-glycol-mono-butyl ether, propylene, or ethylene dichloride, possesses the foregoing combination 45 of properties, thereby rendering it superior to the solvent liquids or liquid mixtures hitherto used in the art and, therefore, particularly well adapted as a wax-precipitating medium for use in the manufacture of low pour test paraffin base lubricating oil. The relative proportion of these liquids to each other, as well as that of the resulting solvent mixture to the oil, may be varied as desired, depending upon the nature of the oil undergoing treatment.

Thus when dewaxing a lubricating distillate 55

fraction, having a viscosity of around 70 to 80 Saybolt universal seconds or higher at 210° F., about thirty parts of the oil may be mixed with about seventy parts of a solvent mixture composed of around 20% ortho-dichloro-benzene and about 80% of a commercial grade amyl alcohol. The resulting mixture is then chilled to about -10° F. or to a temperature corresponding substantially to the desired pour test of the resulting dewaxed oil, following which it is subjected to filtration while still maintained in a cold condition to separate the precipitated wax constituents. Advantageously filtration may be carried out in the presence of a finely divided comminuted filter-aid material which may be added to and commingled with the cold mixture of oil, solvent and suspended wax crystals. After removal of the solvent liquid from the filtrate, the resulting lubricating oil will have a pour test of 0° F. or lower.

Similar results may be obtained, on the other hand, by mixing the oil in about the same proportion with a solvent mixture composed of about 65% ortho-dichloro-benzene and about 35% of either ethylene or propylene dichloride. It is frequently desirable to employ a solvent liquid mixture in which the benzene is at least equal in volume to either the ethylene or propylene dichloride.

While the use of the foregoing solvent liquid mixtures has been described in connection with a lubricating distillate fraction of relatively high viscosity, it is contemplated that mixtures of these solvent liquids may be equally well employed with oils of various viscosity ranges. It is also contemplated that mixtures of these solvent liquids are not necessarily restricted to dewaxing distillate fractions but may also be used in dewaxing various wax-bearing fractions of mineral oil.

Obviously many modifications and variations of the invention, as hereinbefore set forth, may be made without departing from the spirit and scope thereof, and therefore only such limitations should be imposed as are indicated in the appended claims.

We claim:

1. The process of dewaxing wax-bearing oil which comprises mixing with the oil a selective solvent liquid composed of ortho-dichloro-ben-

zene and a mono-alkyl ether of ethylene and diethylene glycol having the wax anti-solvent character and action of ethylene glycol mono-ethyl ether and diethylene glycol mono-butyl ether in such proportions that at temperatures of the order of -10° F. the mixture has substantially complete solvent action on the oil but substantially no solvent action on the wax, chilling the mixture to precipitate the wax, separating the wax thus precipitated, and removing the solvent from the resulting dewaxed oil.

2. The process of dewaxing wax-bearing oil which comprises mixing with the oil a selective solvent liquid composed of ortho-dichloro-benzene and ethylene-glycol-mono-ethyl-ether in such proportions that at temperatures of the order of -10° F. the mixture has substantially complete solvent action on the oil but substantially no solvent action on the wax, chilling the mixture to precipitate the wax, separating the wax thus precipitated, and removing the solvent from the resulting dewaxed oil.

3. The process of dewaxing wax-bearing oil which comprises mixing with the oil a selective solvent liquid composed of ortho-dichloro-benzene and diethylene-glycol-mono-butyl-ether in such proportions that at temperatures of the order of -10° F. the mixture has substantially complete solvent action on the oil but substantially no solvent action on the wax, chilling the mixture to precipitate the wax, separating the wax thus precipitated, and removing the solvent from the resulting dewaxed oil.

4. The process of dewaxing wax-bearing oil which comprises mixing with the oil a selective solvent liquid composed of ortho-dichloro-benzene and a liquid selected from the group consisting of ethylene glycol mono-ethyl ether and diethylene glycol mono-butyl ether in such proportions that at temperatures of the order of -10° F. the mixture has substantially complete solvent action on the oil but substantially no solvent action on the wax, chilling the mixture to precipitate the wax, filtering the cold mixture in the presence of a filter-aid material to remove the wax, and removing the solvent from the resulting dewaxed filtrate.

BERNARD Y. McCARTY.

WILLIAM E. SKELTON.

50